# EUROPEAN PATENT APPLICATION

(11) **EP 4 663 851 A1**
(43) Date of publication of application: **17.12.2025**
(21) Application number: 25182431.4
(22) Date of filing: 12.06.2025
(51) Int. Cl.: E01C 13/08, D06N 7/00

(54) **ARTIFICIAL TURF MAT, METHOD FOR MANUFACTURING AN ARTIFICIAL TURF MAT AND USE OF ARTIFICIAL TURF MAT FOR SPORTS FIELDS**

(30) Priority: 14.06.2024 BE 202405353
(71) Applicant: Sports and Leisure Group NV, 9100 Sint-Niklaas (BE)
(72) Inventor: PENNINCK, John, 9100 Sint-Niklaas (BE)
(74) Representative: Brantsandpatents bv

(57) **Abstract**

The present invention relates to an artificial turf mat comprising a primary backing, with a front side and an opposite rear side; a plurality of filaments of synthetic material, wherein the filaments are tufted onto the primary backing; and a coating, which is located on the back of the primary backing, wherein said filaments have a rounded cross-section, and wherein one or more of the following characteristics are met: a largest cross-sectional dimension of said filaments is less than 250 µm; and/or said filaments comprise a processing aid additive. The invention also relates to a method for manufacturing an artificial turf mat and the use of an artificial turf mat for sports fields, in particular hockey.

## Description

### TECHNICAL FIELD

The invention relates to a device for artificial grass mats. In a second aspect, the invention also relates to a method for manufacturing an artificial turf mat.

### PRIOR ART

Artificial turf mats are known in the prior art for various applications, including for sports fields. Typically, artificial turf mats for use on sports fields, for example hockey fields, need to be irrigated with water before and/or during play on the artificial turf mats, in order to improve their playing characteristics. Such irrigated artificial turf mats are also referred to as water-based pitches.

EP 4321685 describes an artificial turf mat designed for various applications. The artificial turf mat comprises a primary backing with an upper side and a lower side, tufts protruding above the upper side, and a primary coating on the lower side of the primary backing to secure the tufts. Two types of filaments are used in this regard: crimped filaments and substantially straight or spiral-shaped filaments. This plurality of filaments allows for a limited reduction in the friction of the artificial turf mat, thereby improving ball roll movement on the artificial turf mat. The artificial turf mat as described in EP 4321685, however, fails to approximate or equal all playing characteristics of a water-based pitch, for example, with regard to resistance, running comfort, and playing comfort.

AU 2022 305 790 discloses a sports surface comprising loop-shaped pile fibers. To reduce friction and to facilitate managing the need for water irrigation, the loop-shaped pile fibers can remain uncut.

US 2022/025587 describes artificial turf filaments in a core-and-shell structure, comprising polymer particles with different refractive indices to achieve a natural grass-like appearance.

US 2021/404126 describes an artificial turf system that combines primary straight fibers with secondary textured fibers at different heights to create an infill-free playing surface.

The present invention aims to provide at least a solution for some of the above-mentioned problems or disadvantages. The aim of the invention is to provide a method which eliminates those disadvantages.

### SUMMARY OF THE INVENTION

In a first aspect, the present invention relates to an artificial turf mat according to claim 1.

Artificial turf mats for sports fields comprising filaments with a rounded cross-section provide improved flexibility and softness compared to filaments with a non-rounded cross-section. Consequently, a consistent and fast ball roll movement can be obtained on an artificial turf mat according to the invention. Moreover, the artificial turf mats can feel comfortable for players to run and play on. Furthermore, a largest cross-sectional dimension of the filaments of less than 250 µm may contribute to an even higher flexibility compared to filaments merely having a rounded cross-section. In this context, the presence of the processing aid additive is also advantageous. A combination of all these features is advantageous, whereby hardly any or no infill material is required between the filaments.

Preferred embodiments of the artificial turf mat are set forth in claims 2 to 12.

In a second aspect, the present invention relates to a method for manufacturing an artificial turf mat according to claim 13.

The method is advantageous because a combination of sufficient stiffness and sufficient flexibility of the filaments is obtained. Moreover, no infill material is needed on the artificial turf mat.

In a third aspect, the present invention relates to a use of an artificial turf mat according to claim 14. A preferred embodiment of this use is set forth in claim 15.

### DETAILED DESCRIPTION

In a first aspect, the invention relates to an artificial turf mat.

Unless otherwise defined, all terms used in the description of the invention, including technical and scientific terms, have the meaning as commonly understood by a person skilled in the art to which the invention pertains. For a better assessment of the description of the invention, the following terms are explicitly explained.

In this document, "a" and "the" refer to both the singular and the plural, unless the context presupposes otherwise. For example, "a segment" means one or more segments.

The terms "comprise," "comprising," "consist of," "consisting of," "provided with," "include," "including," "contain," "containing," are synonyms and are inclusive or open terms that indicate the presence of what follows, and which do not exclude or prevent the presence of other components, characteristics, elements, members, steps, as known from or disclosed in the prior art.

Quoting numeric intervals by the endpoints includes all integers, fractions, and/or real numbers between the endpoints, including those endpoints.

In the context of the present invention, the term "filaments" is to be interpreted as thin, thread-like structures, which constitute raw materials for the textile industry. In particular, the term "filament" is used for structures of limited length, whereas the term "continuous filament" is used for continuous structures. In the context of the present invention, the term "yarn" is to be understood as a continuous material composed of two or more filaments. Yarn is typically obtained by twisting said two or more filaments. The filaments and yarn as described herein are suitable for use in artificial turf mats according to the present invention.

In the context of this document, "tufting of filaments" means that filaments extend at least partially from a front side of the primary backing. The filaments are thereby at least partially exposed on a rear side of the primary backing in the form of stitch loops.

The artificial turf mat according to the invention comprises a primary backing, with a front side and an opposing rear side; a plurality of filaments made of synthetic material, wherein the filaments are tufted through the primary backing; and a coating, which is located on the rear side of the primary backing.

According to an embodiment, the filaments have a rounded cross-section, and one or more of the following features are present: a largest cross-sectional dimension of the filaments is less than 250 µm, and/or said filaments comprise a processing aid additive.

This embodiment is advantageous for artificial turf mats for sports fields, as the rounded cross-section provides more flexible and softer filaments compared to filaments with a non-rounded cross-section. Consequently, a consistent and fast ball roll movement can be obtained. Moreover, the artificial turf mats can feel comfortable for players to run and play on. Furthermore, the largest cross-sectional dimension of the filaments being less than 250 µm contributes to a higher flexibility compared to filaments that only have a rounded cross-section. Alternatively or in combination with the largest cross-sectional dimension as described herein, the presence of a processing aid additive provides a reduction of frictional resistance at the surface of the fibers, compared to filaments that only have a rounded cross-section.

Preferably, both features are present.

According to an embodiment, the rounded cross-section of the filaments is a polygon with rounded corners. Preferably, the corner radius of the rounded corners is at least 5 µm, more preferably at least 10 µm, more preferably at least 25 µm, more preferably at least 50 µm. Preferably, the corner radius of the rounded corners is at most 150 µm, more preferably at most 125 µm, more preferably at most 100 µm, more preferably at most 75 µm. According to a further or alternative embodiment, the corner radius of the rounded corners is comprised between 5 and 150 µm, between 10 and 125 µm, between 25 and 100 µm, most preferably between 50 and 75 µm.

According to an embodiment, the largest cross-sectional dimension of the filaments is comprised between 75 µm and 250 µm. Preferably, the largest cross-sectional dimension of the filaments is less than or equal to 225 µm, preferably less than or equal to 200 µm. Preferably, the largest cross-sectional dimension of the filaments is greater than or equal to 100 µm, preferably greater than or equal to 150 µm. According to a further or alternative embodiment, the largest cross-sectional dimension of the filaments is comprised between 100 and 225 µm, preferably comprised between 150 and 200 µm. Hereby, an improved stiffness of the filaments can be obtained in combination with sufficient flexibility.

Sufficient stiffness of the filaments may mean that the filaments have an elastic modulus of at least 5 N measured according to EN 13864, preferably with a maximum of 25 N, whereby the filaments retain good flexibility.

According to an embodiment, the smallest cross-sectional dimension of the filaments is comprised between 25 µm and 250 µm. Preferably, the smallest cross-sectional dimension of the filaments is less than or equal to 200 µm, preferably less than or equal to 150 µm. Preferably, the smallest cross-sectional dimension of the filaments is greater than or equal to 50 µm, preferably greater than or equal to 75 µm, preferably greater than or equal to 100 µm. According to a further or alternative embodiment, the smallest cross-sectional dimension of the filaments is comprised between 50 and 200 µm, preferably comprised between 75 and 100 µm. The cross-sectional dimensions described herein contribute to improved UV resistance, in combination with sufficient stiffness of the filaments. UV resistance means that the filaments do not break as a result of degradation from exposure to UV light, which causes the filaments to become brittle from the surface. Sufficient UV resistance is determined by means of weathering tests according to EN 14836, method 2.

According to an embodiment, the processing aid additive is a siloxane additive. The siloxane additive imparts a smoother feel to the filaments, whereby, inter alia, the resistance at a surface of the filaments is reduced. Preferably, the siloxane additive is a nonionic siloxane oil; more preferably, the siloxane additive is a polyether-modified polysiloxane oil. This oil further acts as a lubricant and as a dispersion component. Alternative processing aid additives besides siloxane additive may include: a polyoxyalkylalkene such as polyethylene glycol, or a polyfluoroalkyl such as perfluorooctanoic acid, or a polyacrylate such as poly(ethyl methacrylate). The processing aid additive aims to improve the processing of the extruded filaments during extrusion, whereby, inter alia, die drool is reduced.

According to an embodiment, the processing aid additive has a number-average molecular weight comprised between 1000 g/mol and 50000 g/mol. Preferably, the number-average molecular weight is at least 1500 g/mol, more preferably 2000 g/mol, more preferably 2500 g/mol. Preferably, the number-average molecular weight is at most 35000 g/mol, more preferably at most 20000 g/mol, more preferably at most 5000 g/mol. According to some embodiments, the processing aid additive has a number-average molecular weight comprised between 1500 and 35000 g/mol, preferably between 2000 and 20000 g/mol, more preferably between 2500 and 5000 g/mol. This is advantageous as the migration and volatilization of the processing aid additive during use of the artificial turf mat remains limited within the upper and/or lower limits described herein. On the other hand, migration of the processing aid additive to the surface of the filaments remains possible during production of the filaments.

According to an embodiment, the processing aid additive is present in the filaments in an amount of 0.1 wt% to 10 wt%, where weight percentages are expressed relative to the total weight for making a compound for production of the continuous extruded filaments. Preferably, the processing aid additive is present in an amount of 0.3 wt% to 5 wt%, more preferably 0.5 wt% to 4.0 wt%, more preferably 0.7 wt% to 3 wt%.

According to a further or alternative embodiment, the filaments comprise a microstructure on their surface. The microstructure in the context of the present invention is preferably a microstructure that extends longitudinally along the length of the filament. More preferably, the microstructure is uniform over each cross-section of the filament, perpendicular to the longitudinal axis of the filament. The microstructure may possibly be achieved by extrusion through a die plate comprising openings which form the microstructure on their circumferential edge.

According to an embodiment, the microstructure comprises a sinusoidal pattern. Preferably, this sinusoidal pattern extends longitudinally along the length of the filament. More preferably, this sinusoidal pattern is uniform over each cross-section of the filament, perpendicular to the longitudinal axis of the filament. According to some embodiments, the sinusoidal pattern has an amplitude comprised between 1 µm and 25 µm, preferably between 2 µm and 20 µm, more preferably 3 µm and 15 µm, even more preferably 4 µm to 10 µm. According to some embodiments, the amplitude of the sinusoidal pattern is at least 1.5 µm, preferably at least 2.5 µm, more preferably at least 3.5 µm. According to some embodiments, the amplitude of the sinusoidal pattern is at most 12.0 µm, preferably at most 9.0 µm, more preferably at most 6.0 µm.

According to some embodiments, the sinusoidal pattern has a wavelength comprised between 1 µm and 50 µm, preferably between 2 µm and 25 µm, more preferably between 3 µm and 15 µm. According to some embodiments, the wavelength of the sinusoidal pattern is at least 2 µm, preferably at least 4 µm, more preferably at least 6 µm, more preferably at least 8 µm, more preferably at least 10 µm. According to some embodiments, the wavelength of the sinusoidal pattern is at most 40 µm, preferably at most 30 µm, more preferably at most 20 µm, more preferably at most 10 µm.

The wavelength and amplitude of the sinusoidal pattern as described herein contribute to a ball roll distance of at least 8.5 ± 0.5 m. Due to the lower friction, a ball can roll further with the same applied force. This is due to the increased flexibility of the filaments. The ball roll distance is determined according to the standards of the International Hockey Federation for dry artificial turf mats. Moreover, the microstructure of the filaments contributes to a shock-absorbing effect.

According to an embodiment, the cross-section of the filaments is elliptical. Preferably, the cross-section of the filaments is circular. Owing to the elliptical, preferably circular, cross-section of the filaments, an improved balance can be obtained between stiffness and flexibility of the filaments. Preferably, a ratio of the longest diameter to the shortest diameter of the elliptical cross-section is at most 2, more preferably at most 1.5, more preferably at most 1.3, more preferably at most 1.1. Even more preferably, said ratio is at least 1.

According to an embodiment, a number of tufts per unit area of the artificial turf mat is at least 60,000 tufts/m² and at most 100,000 tufts/m². Preferably, a number of tufts per unit area is at least 63,000 tufts/m², more preferably at least 66,000 tufts/m², more preferably at least 69,000 tufts/m², more preferably at least 71,000 tufts/m². Preferably, a number of tufts per unit area is at most 97,000 tufts/m², more preferably at most 94,000 tufts/m², more preferably at most 91,000 tufts/m², more preferably at least 88,000 tufts/m², more preferably at least 85,000 tufts/m². According to some embodiments, the number of tufts per unit area of the artificial turf mat is comprised between 63,000 and 97,000 tufts/m², preferably comprised between 66,000 and 94,000 tufts/m², more preferably comprised between 69,000 and 91,000 tufts/m², even more preferably between 71,000 and 85,000 tufts/m². Due to the presence of at least 60,000 tufts/m², there is sufficient coverage so that the primary backing is not visible and can provide sufficient shock absorption. Moreover, a tuft density of at most 100,000 tufts/m² allows sufficient movement of the tufts. A further advantage is that the filaments are thereby more wear-resistant.

According to an embodiment, the tufts are uniformly distributed over the primary backing. "Uniformly" is preferably to be understood to mean that when subdividing the primary backing into smaller sections, each of these sections has the same number of tufts per unit area.

According to an embodiment, the portion of the filaments, which extends from the primary backing, preferably from the front side of the primary backing, to the distal end of the filaments, has a length of at least 8 mm and at most 15 mm. Preferably, the length is at most 14.5 mm, more preferably at most 14.0 mm, more preferably at most 13.5 mm, more preferably at most 13.0 mm. Preferably, the length is at least 8.0 mm, more preferably at least 8.2 mm, more preferably at least 8.5 mm. According to some embodiments, the portion of the filaments which extends from the primary backing to the distal end of the filaments has a length comprised between 8.0 and 14.5 mm, preferably comprised between 8.2 and 14.0 mm, more preferably comprised between 8.5 and 13.5 mm, most preferably between 8.5 and 13.0 cm. Due to the length of the filaments of at least 8 mm and at most 15 mm, the filaments can remain upright if there is no compression of the filaments. At the same time, there is sufficient flexibility of the filaments without folds being able to form in the filaments. Moreover, shorter filaments provide a lower resistance to ball roll movement. The length as described herein contributes to a further improvement of stiffness and flexibility of the filaments.

According to an embodiment, a filament is a segment of a continuous filament. According to some embodiments, the filament has a length of at least 17 mm and at most 30 mm. Preferably, the filament has a length of at least 19 mm, more preferably at least 21 mm. Preferably, the filament has a length of at most 28 mm, more preferably at most 26 mm. According to some embodiments, the filament has a length comprised between 19 and 28 mm, preferably comprised between 21 and 26 mm.

According to an embodiment, the artificial turf mat comprises no infill material. In prior art artificial turf mats, sand, elastic particles, whether foamed or not, or water are typically used for keeping the filaments upright, i.e., as infill material. According to some embodiments, the artificial turf mat may comprise one or more infill materials. Thus, functionalities such as shock absorption can possibly be further improved.

According to an embodiment, the filaments comprise a polyolefin. Preferably, the polyolefin is a low-density polyethylene. More preferably, the polyolefin is a linear low-density polyethylene and/or a linear very-low-density polyethylene. Alternatively, the polyolefin is a polypropylene, more preferably a copolymer polypropylene, even more preferably an impact copolymer polypropylene. Another alternative is that a combination of polyethylene and polypropylene filaments is used, from which the tufts are formed.

Polyolefins are easy to maintain because they are naturally antifungal and antibacterial, water-resistant, and have good resilience. The polyolefin filaments can also be easily recycled in the same or a different application.

According to an embodiment, the artificial turf mat comprises ethyl vinyl acetate, polyamide, polystyrene, polyvinylidene fluoride, high-density polyethylene, medium-density polyethylene, low-density polyethylene, linear low-density polyethylene, very low linear density polyethylene, anhydride-modified polyethylene, polypropylene, polyethylene, polyester, polyamide, or a combination thereof. Said polyamide is preferably a polylaurolactam or a polycaprolactam. The aforementioned polyamide is preferably a polylaurolactam or a polycaprolactam.

According to an embodiment, the filaments are monofilaments, wherein each tuft is a combination of 8 to 16 monofilaments, preferably 10 to 14 monofilaments, more preferably 12 monofilaments. More preferably, each tuft is a combination of at least 9 monofilaments, preferably at least 11 monofilaments. Preferably, each tuft is a combination of at most 15 monofilaments, preferably at most 13 monofilaments. Between 8 to 16 monofilaments per tuft ensures that the filaments in each tuft can fan out sufficiently, whereby the filament provides coverage over the artificial turf mat and the primary backing is not visible. "Fanning out" means in the context of the invention that the filaments are located substantially apart from each other with their free, distal ends.

According to an alternative embodiment, the filaments are made from a thin sheet that is cut into filaments. Preferably, the thin sheet is biaxially stretched.

According to an embodiment, the filaments comprise a UV additive. Preferably, the UV additive is a UV absorber, a hindered amine light stabilizer, an antioxidant, or a combination thereof, whereby the filaments are more UV-resistant than without the UV additive. Preferably, the UV additive is comprised in the filaments in 0.1 wt% to 1.0 wt%.

According to an embodiment, the filaments comprise a filler. Preferably, the filler is calcium carbonate, more preferably, the calcium carbonate is micronized. The filler contributes to a microstructure on the surface of the filaments and can additionally contribute to antiblocking properties of the filaments with respect to each other. Preferably, the filler is incorporated in the filaments in 0.3 wt% to 1.0 wt%.

According to an embodiment, the tufts of the artificial turf mat have a yarn density of at least 4000 dtex and at most 10000 dtex. Dtex is a measure of linear mass density of filaments and is defined as the weight in grams per 10,000 meters. Preferably, the yarn density is at least 5000 dtex, more preferably at least 6000 dtex. Preferably, the yarn density is at most 7500 dtex, more preferably at most 7000 dtex. According to some embodiments, the tufts of the artificial turf mat have a yarn density comprised between 5000 and 7500 dtex, preferably comprised between 6000 and 7000 dtex. The yarn density as described herein allows tufts to fan out with sufficient space, whereby the filaments can move flexibly, but at the same time connect sufficiently closely to each other so that the filaments can support each other in an upright position.

According to an embodiment, the artificial turf mat comprises between 1 and 3 million filaments per square meter. Preferably at least 1.5 million filaments per square meter and at most 2.5 million filaments per square meter. Preferably, the artificial turf mat comprises at least 1.6 million filaments/m², more preferably at least 1.7 million filaments/m². Preferably, the artificial turf mat comprises at most 2.2 million filaments/m², more preferably at most 2.0 million filaments/m². According to some embodiments, the artificial turf mat comprises between 1.6 and 2.2 million filaments per square meter, preferably between 1.7 and 2.0 million filaments per square meter. As a result of the high number of filaments per square meter, an increased density of the artificial turf mat is obtained, whereby a more consistent and stable playing surface is obtained. Moreover, the risk of injuries for the players is reduced because the playing surface is softer. Preferably, the filaments are monofilaments.

According to an embodiment, the artificial turf mat has a pile weight of at least 1000 g/m², preferably of at least 1500 g/m², more preferably of 2000 g/m², and the artificial turf mat has a pile weight of at most 3500 g/m². The term "pile weight" in the context of the present invention refers to the total weight of the filaments used per square meter of the artificial turf mat. Due to short filaments with a length of at most 15 mm, the pile weight is low, which simplifies placement of the artificial turf mats. Additionally, the pile weight gives an indication of the number of tufts and the number of filaments per unit area.

According to one embodiment, the primary backing includes a fiberglass mat. Preferably, the primary backing comprises one to three layers of woven or non-woven textile. The textile can be made of polypropylene, polyester, or other synthetic materials. More preferably, the primary backing is a woven polyolefin fabric, whereby recycling of the artificial turf mat is simplified. Preferably, the primary backing consists of three layers wherein the outer layers comprise a woven and/or non-woven material and the middle layer comprises a dimensionally stabilizing woven or non-woven material, such as, for example, the fiberglass mat. Due to the fiberglass mat, the primary backing obtains a reinforced form, whereby fatigue of the primary backing due to deformation is considerably reduced.

According to an embodiment, the primary backing has a weight comprised between 250 g/m² and 500 g/m². Preferably, the primary backing has a weight of at least 300 g/m², more preferably of at least 350 g/m². Preferably, the primary backing has a weight of at most 450 g/m², more preferably of at least 400 g/m².

According to an embodiment, the coating is a latex, a polyurethane elastomer, or a polyolefin dispersion. Preferably, the coating is a synthetic latex comprising a polyolefin. Alternatively, the backing is a polyolefin dispersion comprising an ethylene-propylene rubber. These materials are particularly advantageous as a coating as they are easy to apply and effect a good fixation of the filaments. Furthermore, the abovementioned materials are advantageous during recycling; in particular, they allow for easy separation of the coating and the filaments.

According to an embodiment, the coating has a mass per square meter comprised between 300 g/m² and 2000 g/m², preferably comprised between 500 g/m² and 1500 g/m², more preferably comprised between 700 g/m² and 1200 g/m².

According to an embodiment, the rotational resistance of the artificial turf mat is between 25 and 50 Nm, measured according to standard EN 15301-1. This ensures that the artificial turf mat provides sufficient grip for users, so that users do not slip. This consequently prevents injuries. According to an embodiment, the vertical deformation of the artificial turf mat is 4 mm to 9 mm, measured according to standard EN 14809.

According to an embodiment, the artificial turf mat comprises an underlay. The underlay preferably lies against the back of the primary backing, as a substructure on the coating and provides additional strength to the artificial turf mat. The underlay is preferably moisture-permeable, shock-absorbing and/or acoustically insulating. More preferably, the underlay is attachable to the underside of the coating or the underlay, even more preferably attachable during installation of the artificial turf mat. According to some embodiments, the underlay is foamed; preferably, the underlay is a polyolefin foam or a polyurethane foam.

As an alternative to a tufted artificial turf mat, according to alternative embodiments of the invention, the artificial turf mat is a woven mat, a needle-felted mat, a knitted mat, or a mat produced using a velour technique. The filaments incorporated in the artificial turf mat have rounded cross-sections. Moreover, one or more of the following features are met: the largest cross-sectional dimension of the filaments is less than 250 µm, and/or said filaments comprise a processing aid additive. To one skilled in the art of mats, it will be apparent that the above-mentioned features of the filaments for making the tufts are likewise applicable to the filaments used in woven, needle-felted, knitted or mats produced using a velour technique.

In a second aspect, the invention relates to a method for manufacturing an artificial turf mat.

According to some embodiments, the method comprises the steps of: providing a primary backing, having a front side and an opposite rear side, a plurality of filaments made of synthetic material, and a coating; tufting said filaments through the primary backing, preferably the front side of the primary backing; fixing said filaments by means of applying and curing the coating on the rear side of the primary backing.

According to an embodiment, the filaments have a combination of a rounded cross-section, a largest cross-sectional dimension of the filaments that is less than 250 µm, and the filaments comprising a processing aid additive. This is advantageous because a sufficient stiffness in combination with sufficient flexibility of the filaments is obtained. Additionally, no infill material is needed on the artificial turf mat.

According to an embodiment, the underlay is laminated to the coating during curing.

According to an embodiment, for forming the filaments, the filaments are extruded from a compound, cold-drawn, and finished with several sequential annealing and drawing steps.

In a third aspect, the invention relates to a use of an artificial turf mat for sports fields.

According to an embodiment of this use, the sports fields are hockey fields. There is no infill material present between the tufts on the artificial turf. The combination of several features of the artificial turf mat allows a sufficient stiffness of the filaments to be obtained such that they can remain upright independently and support each other. The filaments also exhibit a reduced frictional resistance, resulting in increased playing comfort for players. Moreover, this artificial turf mat does not require irrigation for playing hockey.

To a person skilled in the art of manufacturing artificial turf mats, more specifically in manufacturing artificial turf mats for sports fields, it is clear that the artificial turf mat according to the first aspect is preferably manufactured according to a method according to the second aspect, and that this artificial turf mat is preferably used according to the third aspect.

In a fourth aspect, the invention relates to the use of filaments as described in preceding aspects for producing mats other than artificial turf mats. The several features of the filaments as described in preceding aspects are also applicable to the use according to the fourth aspect.

Herein, the filament is used in a woven mat, in a needle-felted mat, in a knitted mat, and/or in a mat produced using a velour technique. Said filament preferably has a rounded cross-section. Preferably, one or more of the following features are met: the largest cross-sectional dimension of said filament is less than 250 µm, said filament comprises a processing aid additive and/or the surface of the filament comprises a microstructure. To a person skilled in the technical field of mats, it is clear that the above-mentioned features of the filaments for making tufts for artificial turf mats may also be applicable to the filaments used in woven mats, needle-felted mats, knitted mats or mats produced using a velour technique.

Hereinafter, the invention is described by way of non-limiting examples or figures which illustrate the invention, and are not intended or to be interpreted as limiting the scope of the invention.

### EXAMPLES

The invention will now be further elucidated by means of the following examples, without, however, being limited thereto.

### EXAMPLE 1

Example 1 concerns an artificial turf mat comprising a plurality of filaments, a primary backing and a coating; for sports fields with the features below:

| **filament** | |
|---|---|
| cross section | Elliptical with ratio 1.2 |
| largest cross-sectional dimension | 196-242 µm |
| smallest cross-sectional dimension | 104-135 µm |
| microstructure amplitude | 0.5 ± 0.1 mm |
| microstructure wavelength | 1.3 ± 0.2 mm |
| length | 15 mm |
| synthetic material | linear low-density polyethylene |
| additives | siloxane additive 3 wt%* |
| | |

| **artificial turf mat** | |
|---|---|
| filaments | |
| tufts per square meter | 73,120 tufts/m² |
| filaments per tuft | 12 |
| number of filaments per square meter | 1,754,880 filaments/m² |
| yarn density | 5000 dtex |
| primary backing | |
| first layer | woven polypropylene |
| second layer | fiberglass mat |
| coating | |
| synthetic material | latex |
| mass per square meter | 1200 g/m² |

| | |
|---|---|
| *weight percent relative to total weight compound for making filaments | |

### EXAMPLE 2

Example 2 concerns an artificial turf mat comprising a plurality of filaments, a primary backing and a coating; for sports fields with the features below:

| **fiber** | |
|---|---|
| cross section | round |
| largest cross-sectional dimension | 188-203 µm |
| smallest cross-sectional dimension | 196-206 µm |
| microstructure amplitude | 0.9 ± 0.2 mm |
| microstructure wavelength | 2.1 ± 0.1 mm |
| length | 75 wt%°: 13 mm, 25 wt%°: 10 mm |
| synthetic material | low-density polyethylene |
| additives | siloxane additive 2.5 wt%*, |
| | UV additive 0.2 wt%* |
| | |

| **artificial turf mat** | |
|---|---|
| filaments | |
| tufts per square meter | 79,560 tufts/m² |
| filaments per tuft | 9 |
| number of filaments per square meter | 1,432,080 filaments/m² |
| primary backing | |
| foam thickness | 6 mm |
| synthetic material additional layer | thermoplastic polyurethane elastomer |
| thickness additional layer | 15.5 mm |
| yarn density | 5500 dtex |
| first layer | non-woven polypropylene with long glass fibers |
| coating | |
| synthetic material | polyurethane elastomer |

| | |
|---|---|
| ° weight percentage relative to the total weight of the filaments *weight percentage relative to total weight of the compound for making filaments. | |

### EXAMPLE 3

Example 3 concerns an artificial turf mat comprising a plurality of filaments, a primary backing and a coating, with a separate shock-absorbing foamed underlay; for sports fields with the features below:

| **fiber** | |
|---|---|
| cross section | rounded hexagonal R45 µm |
| largest cross-sectional dimension | 173-191 µm |
| smallest cross-sectional dimension | 112-184 µm |
| microstructure amplitude | 0.9 ± 0.1 mm |
| microstructure wavelength | 1.8 ± 0.1 mm |
| length | 12 mm |
| synthetic material | 65% of the total number of filaments linear low-density polyethylene and 35% impact copolymer polypropylene |
| additives | 0.5 wt% calcium carbonate |
| | 1 wt% polyethylene glycol* |

| | |
|---|---|
| **artificial turf mat** | |
| filaments | |
| tufts per square meter | 84,980 tufts/m² |
| filaments per tuft | 14 |
| number of filaments per square meter | 2,379,440 filaments/m² |
| primary backing | |
| yarn density | 6000 dtex |
| first layer | woven polypropylene |
| second layer | glass filament mat |
| third layer | woven polyethylene |
| coating | |
| synthetic material | polyolefin dispersion |
| mass per square meter | 856 g/m² |

## Claims

1. An artificial turf mat comprising a primary backing, having a front side and an opposite rear side; a plurality of filaments of synthetic material, wherein the filaments are tufted onto the primary backing; and a coating, which is located on the back of the primary backing, **characterized in that** said filaments have a rounded cross-section, and wherein one or more of the following features are present:
- a largest cross-sectional dimension of said filaments is less than 250 µm; and/or
- said filaments comprise a processing aid additive.

2. Artificial turf mat according to claim 1, **characterized in that** said filaments comprise a microstructure on their surface.

3. Artificial turf mat according to claim 1 or 2, **characterized in that** a number of tufts per unit area is at least 60,000 tufts/m² and at most 100,000 tufts/m².

4. Artificial turf mat according to any of the preceding claims 1-3, **characterized in that** the portion of the filaments, which extends from the primary backing, preferably from the front side of the primary backing, to the distal end of the filaments has a length of at least 8 mm and at most 15 mm.

5. Artificial turf mat according to any of the preceding claims 1-4, **characterized in that** said filaments comprise a polyolefin, preferably linear low-density polyethylene.

6. Artificial turf mat according to any of the preceding claims 1-5, **characterized in that** said filaments are monofilaments, where each tuft is a plurality of 8 to 16 monofilaments.

7. Artificial turf mat according to any of the preceding claims 1-6, **characterized in that** the cross-section of said filaments is elliptical, wherein a ratio of the longest diameter to the shortest diameter of the elliptical cross-section is at most 2.

8. Artificial turf mat according to any of the preceding claims 1-7, **characterized in that** the tufts of the artificial turf mat have a yarn density of at least 4000 dtex and at most 10,000 dtex.

9. Artificial turf mat according to any of the preceding claims 1-8, **characterized in that** the artificial turf mat comprises between 1 and 3 million filaments per square meter.

10. Artificial turf mat according to any of the preceding claims 1-9, **characterized in that** the artificial turf mat has a pile weight of at least 1000 g/m².

11. Artificial turf mat according to any of the preceding claims 1-10, **characterized in that** the primary backing comprises a glass filament mat.

12. Artificial turf mat according to any of the preceding claims 1-11, **characterized in that** the coating is a latex, a polyurethane elastomer or a polyolefin dispersion.

13. Method for manufacturing an artificial turf mat, wherein the method comprises the steps of: providing a primary backing, having a front side and an opposite rear side, a plurality of filaments of synthetic material, and a coating; tufting said filaments through the primary backing, preferably the front side of the primary backing; fixing said filaments by spreading and curing the coating on the rear side of the primary backing; **characterized in that** the artificial turf mat is an artificial turf mat according to claims 1-12.

14. Use of an artificial turf mat for sports fields, **characterized in that** the sports fields are hockey fields, wherein no infill material is present between the tufts.

15. Use of an artificial turf mat for sports fields according to claim 14, **characterized in that** the artificial turf mat is an artificial turf mat according to any of the preceding claims 1-12.
